# EUROPEAN PATENT APPLICATION

(11) **EP 1 433 900 A2**
(43) Date of publication of application: **30.06.2004**
(21) Application number: 03013539.6
(22) Date of filing: 13.06.2003
(51) Int. Cl.: E01B 19/00

(54) **Noise and vibrating reducing railway pad**

(30) Priority: 18.12.2002 GB 0229388
(71) Applicant: Sugden, Vincent, Poynton, Cheshire SK12 1NU (GB); Phillips, Roland, Macclesfield, Cheshire (GB); Kuras, Laurence, Grains Bar, Oldhom OL1 4SU (GB)
(72) Inventor: Sugden, Vincent, Poynton, Cheshire SK12 1NU (GB); Phillips, Roland, Macclesfield, Cheshire (GB); Kuras, Laurence, Grains Bar, Oldhom OL1 4SU (GB)

(57) **Abstract**

An attachable pad, which is produced by blending polymeric binders with hard particles is manufactured in a mould whose shape is that which mirrors a railway track.

Attaching these pads to the railway track using mechanical or chemical fixing, reduces the vibration of the track as a train passes over, which in turn reduces the incident noise pollution. The pads can be different heights to allow maintenance work on the track without removing the pads.

To further reduce the noise pollution, the pads can be porous which acts as a sound absorber, thus the combination of vibration and sound attenuation gives better results than theory suggests.

## Description

The quietening of railways is currently under examination, especially where railways and population densities come together. Often described as incident noise pollution. The sound of railway wheels on rail track causes a high level of incident noise which in these enlightened days is not acceptable, whereas costs verses lifestyle improvement is becoming more so. The removing of tracks and relaying energy absorbant tracks is too expensive, so outlined below in this invention is a method of reducing the incident noise from railway track whilst keeping costs verses lifestyle improvement to a reasonable acceptable ratio..

According to our invention, by attaching a sound/energy absorbing pad (Qpad) to the side of the railway track, sufficient incidental noise/vibrations will be removed to leave the residue of the noise at an acceptable level.

The pads are a combination of binding agents and hard particulate solids as outlined in our patent application No GB 0128960.2 They can be produced by blending hard particulates preferably sand, flint and other suitably hard aggregates and products like crushed glass or recycled glass with binders such as polyurethanes, silicon resins, polysulphide resins, acrylic, epoxy resins and co-polymers of the above resins, such as epoxy-polysulphide or epoxy-urethane. Other binders for this process can be inorganic types such as sodium silicates, potassium silicates and combinations of both with polyurethane isocyanates These binders are usually mixed in the ratio of 2 - 35%, but more specifically 4 - 12% by weight. The products are weighed into a force type mixer, typically a cumflow mixer and blended together. The product is then placed into individual moulds, cast sheet or continuously extruded, then cut, if needed, into the correct dimensions, i.e. Those that suit the relevant tracks.

To increase the degree of contact of the pad onto the rail a separate layer of the flexible binder with or without aggregate can be added to the inside of the pad , this can be added at the casting stage by laying any of the binders into the mould to partially cure before casting the binder / aggregate blend on top . The more flexible layer can also be added in a post casting process by painting, pouring or spraying onto the face of the pad which will come into cotact with the rail .

The length of each pad can be from 10centimeters to 25 meters cut to length to suit each type of track, but usually 40centimeters to 1 meter in length. The pads can be attached to the tracks by using metal clips, mechanical fastenings through the pad onto the track or by adhesives such as used to bind the particles of aggregate, I.e. epoxy, polyurethane etc.

### Examples.

### Example 1.

9.5kg Flintag6 is blended with 0.5kg Alpha 4100 polyurethane resin in a mixing bowl and mixed. The blended aggregate/binder is then placed into a 3mm mild steel mould and left until fully cured. The resulting pad when adhered to a metal rail using Alpha 4100 reduces the frequency residence time by 64% over a rail which is unpadded. i.e. when a metal rail is struck with a metal hammer, the rail will vibrate. The vibration and the sound attenuation and resonance is greatly reduced with a pad adhered.

### Example 2.

9.6kg sand Hardcastle 20/40 is blended with 0.4kg Alpha 6100 aliphatic polyurethane resin in a mixer. Once mixed the product is placed in a PVC vacuum form mould until the product has cured, around 24 hours, then de-moulded. When attached to a rail, using method 2 the frequency resonance time is reduced by 36% over the same rail without the pad .

### Example 3 .

Into the mould 0.3kg of Alpha 6100 is poured left for 30 minutes at 25 centigrade then a blend of example 2 is layed on top of the curing polyurethane resin and left for 24 hours when the duel layer pad is attached to rail as per drawing 2 the frequency resonance time is reduced by 73%.

## Claims

1. Producing a pad in example (1), a semi rigid energy absorbing product is formed

2. When attaching the pad as in drawing (1), the noise transmitted through a railway line is much reduced.

3. When attaching the pad as in drawing (2), the noise created by the railway line is much reduced

4. When attaching the pad as in drawing (3), the incidental noise pollution is very much reduced

5. When attaching the pad as is in drawing (1), (2), & (3) the transmitted noise, created noise and incidental noise pollution are very much reduced.
